

3,440,226

## POLYCARBONAMIDES RESISTANT TO ACID DYES

Lawrence W. Crovatt, Jr., Raleigh, N.C., and William A. H. Huffman, deceased, late of Durham, N.C., by Ernestine H. Huffman, executrix, Antioch, Tenn., assignors to Monsanto Company, St. Louis, Mo., a corporation of Delaware

No Drawing. Filed Oct. 21, 1965, Ser. No. 502,777  
Int. Cl. C08g 20/38; D01f 7/04

U.S. Cl. 260—78

11 Claims 10

### ABSTRACT OF THE DISCLOSURE

Fiber-forming linear polycarbonamides modified to contain certain terminal naphthyl disulfonated radicals as an integral part of the polymer chain possess excellent acid dye-resistant properties. Fibers formed from these polycarbonamides may, for example, be combined with standard polycarbonamide fibers to provide a fabric which is dyeable in a single dye bath to different colors or color tones.

This invention relates to fiber-forming synthetic polymeric materials and the shaped articles produced therefrom. More particularly, this invention relates to novel fiber-forming synthetic linear polycarbonamides and shaped articles produced therefrom which are particularly resistant to acid type dyes.

Although textile fibers obtained from fiber-forming polycarbonamides heretofore known are of great value, they are deficient in dying properties in that they all possess the same acid dyeable characteristic and each type will dye to a single shade only. This is a distinct disadvantage since it eliminates the possibility of obtaining other desirable color effects where some of the fibers do not absorb dye or absorb less dye. It is desirable therefore, to produce polycarbonamides which have acid dye resist characteristics so that by combining such polycarbonamides with standard polycarbonamides in varying amounts it would be possible to produce polycarbonamide articles which are dyeable to different tones of the same color.

Heretofore, additives employed for this purpose have not been found to be entirely satisfactory due to their ability to impart only a limited amount of acid dye-resistance to the fibers. For example, U.S. Patent No. 3,039,990 discloses fibers with alkali metal dicarboxybenzene monosulfonates. While these additives serve to make the fibers receptive to basic dyes, they do not impart a sufficient acid dye-resist character to the fibers to make them commercially acceptable for use with acid dyes in the production of a wide range of off-shade fabrics.

It is an object of the present invention to provide novel and useful fiber-forming synthetic linear polycarbonamides.

Another object is to provide shaped articles such as textile fibers, produced from such polycarbonamides, the said article having superior acid dye-resist properties. A further object is to provide a process for the production of polycarbonamides from which shaped articles having superior acid dye-resist properties can be prepared.

These and other objects will become apparent in the course of the following specification and claims.

The polycarbonamides of the present invention are useful in the production of shaped articles by extrusion, molding, or casting in the nature of yarns, fabrics, films, pellicles, bearings, ornaments, or the like. They are particularly useful in the production of textile fibers.

The present invention provides a novel polycarbonamide wherein recurring carbonamide linkages are an integral part of the polymer chain and containing as a

component part of the polymer chain between about 0.05 and 2.0 mole percentage and preferably between about 0.1 and about 1.0 mole percentage, based on the molecular weight of the polycarbonamide, of units of the structure:



wherein Z is a member of the class consisting of



and



20 X is a member of the class consisting of hydrogen and lower alkyl, M is a member of the class consisting of hydrogen, the ammonium radical and an alkali metal and n is a number from zero to 6 inclusive with the proviso that when Z is



then n is at least 1.

As used herein, the term "molecular weight of the polycarbonamide" refers to the molecular weight of one repeating unit of the polycarbonamide. Thus, the molecular weight of polyhexamethylene adipamide would be 226 which is the molecular weight of one repeating unit having the formula



In a typical preparation the polycarbonamide is formed by interpolymerizing a polycarbonamide composition selected from the group consisting of (A) substantially equimolecular proportions of a dibasic carboxylic acid having the formula:



45 wherein R is a divalent hydrocarbon radical, and a diamine having the formula:



50 wherein X and R are as defined above, and (B) a monoaminomonocarboxylic acid having the formula:



55 wherein X and R are as defined above, in the presence of a monofunctional disulfonated compound having the formula:



wherein n, Z and M are as defined above and Y is a member of the class consisting of hydrogen, —OH, —CL and OR', R' being a monovalent hydrocarbon radical such that R'—OH is volatile below the decomposition temperature of the polycarbonamide formed.

The nature of the radical —R— in the acid, the diamine, or the aminoacid is not critical. Preferably, it is a divalent hydrocarbon radical containing no more than about 20 carbon atoms. Typical acids of the class il-

Illustrated by the formula designated (b) are oxalic, adipic, suberic, pimelic, azelaic, sebacic, brassylic, octadecanedioic, undecanedioic, glutaric, tetradecanedioic, p-phenylene diacetic, isophthalic, terephthalic, hexahydroterephthalic, and the like, and mixtures thereof.

Typical suitable diamines of the class illustrated by the formula designated (c) above are ethylene diamine, propylene diamine, tetramethylene diamine, pentamethylene diamine, hexamethylene diamine, octamethylene diamine, decamethylene diamine, p-xylylenediamine, p-phenylenediamine, hexahydro - p - phenylenediamine, bis(4 - aminocyclohexyl)methane, piperazine, dimethylpiperazine, tetramethylpiperazine, the N,N'-dimethyl, the N,N'-diethyl and the N,N'-diisopropyl derivatives of the above, and the like, as well as mixtures thereof.

Typical suitable amino acids of the class represented by the formula designated (d) above are 6-aminocaproic acid, 9-aminononanoic acid, 11-aminoundecanoic acid and 17-aminoheptadecanoic acid.

In place of the above noted dibasic carboxylic acids, diamines, and amino acids, the amide-forming derivatives thereof can be employed to form fiber-forming polymers. Amide-forming derivatives of the dibasic carboxylic acids comprise the mono- and di-ester, the anhydride, the mono- and di-amide and the acid halide. Amide-forming derivatives of the diamines include carbamate and the N-formyl derivative. Amide-forming derivatives of the amino acids include the ester, anhydride, amide, lactam, acid halide, N-formyl derivative, carbamate, and, in the presence of water, the nitrile.

As indicated above the compounds found useful in the practice of this invention are characterized by two sulfonate groups and one amide-forming group attached to a naphthalene ring and are represented by the formula:



wherein n, Z, M and Y are as defined above. Illustrative of such compounds when



are: di(potassium sulfonate) - naphthalene - 2 - carboxylic acid, di(ammonium sulfonate) - naphthalene - 2 - carboxylic acid, di(potassium sulfonate) - naphthalene - 1 - carboxylic acid, di(sulfonic acid) - naphthalene - 2 - carboxylic acid, di(potassium sulfonate) - naphthalene - 2 - ethanoic acid, di(ammonium sulfonate) - naphthalene - 1 - propionic acid, di(sodium sulfonate) - naphthalene - 2 - pentanoic acid, and di(sulfonic acid) - naphthalene - 1 - heptanoic acid; and when



Illustrative compounds are di(potassium sulfonate) - naphthalene - 2 - methylamine, di(ammonium sulfonate) - naphthalene - 2 - methylamine, di(sulfonic acid) - naphthalene - 2 - ethylamine, di(potassium sulfonate) - naphthalene - 1 - ethylamine, and di(sodium sulfonate) - naphthalene - 2 - pentylamine.

The polycarbonamides of this invention are prepared by procedures well known in the art and commonly employed in the manufacture of simple polyamides. That is, the reactants are heated at a temperature of from 180° C. to 300° C. and preferably from 200° C. to 295° C. until the product has a sufficiently high molecular weight to exhibit fiber-forming properties, which properties are reached when the polyamide has an intrinsic viscosity of at least 0.4. The reaction can be conducted at super-atmospheric, atmospheric, or sub-atmospheric pressure. Often it is desirable, especially in the last stage of the

reaction, to employ conditions, e.g. reduce pressure, which will aid in the removal of the reaction by-products. Preferably, the reaction is carried out in the absence of oxygen, for example, in an atmosphere of nitrogen.

5 Intrinsic viscosity as employed herein is defined as

$$C \xrightarrow{\text{Lim.}} 0 \left( \frac{\log_e N_r}{C} \right)$$

in which N<sub>r</sub> is the relative viscosity of a dilute solution 10 of the polymer in m-cresol in the same units at the same temperature, and C is the concentration in grams of polymer per 100 cc. of solution.

The amount of additive which may be present as a component part of the polymer chain of the polycarbon- 15 amides of this invention may vary depending upon the type of polymer desired and the particular shaped article in which it is to find its end use. It has been found necessary to employ between about 0.05 and 2.0 mole percent- 20 age based on the molecular weight of the polycarbon- amide. At least 0.05 mole percentage of additive is required in order that a significant level of acid dye-resist 25 properties be obtained. It has been found that the best results are obtained when between about 0.1 and about 1.0 mole percentage of additive based on the molecular weight of the polycarbonamide are employed. Amounts greater than 2.0 mole percentage have an adverse effect on the viscosity of the polycarbonamide produced. Since the additives employed in this invention contain only one functional group, i.e., one carboxyl or one amino group,

30 it can be seen that they react in such a manner as to terminate the polymer chain of the polycarbonamide. This type of reaction is similar to the reaction which occurs upon the addition of additives which are termed by the art as chain terminators or viscosity stabilizers. 35 Thus, the greater amount of additive which is employed in the present invention, the shorter will be the polymer chain of the polycarbonamide and the lower will be the viscosity of the polycarbonamide. As noted above, it has been found preferable to employ amounts of additives 40 between about 0.1 and 1.0 mole percentage since when employing such amounts the polycarbonamide produced has been found to possess excellent acid dye-resist properties and to have a viscosity in the fiber-forming range.

In order to illustrate the invention and the advantages 45 thereof with greater particularity, the following specific examples are given; it is to be understood that they are intended to be only illustrative and not limitative. Parts are given by weight unless otherwise indicated.

#### EXAMPLE I

50 This example illustrates preparation of a conventional polycarbonamide namely, polyhexamethylene adipamide. This polymer and the fiber therefrom are to be used as a standard of comparison with the modified polycarbon- 55 amides of the present invention.

To a stainless steel evaporator there was added 8.47 moles of water containing 0.562 mole of hexamethylene diammonium adipate salt dissolved therein. The unit was purged with nitrogen and then pressurized to 13 pounds per square inch gauge. The salt solution was then heated to 137° C. with continuous removal of steam condensate. At this point the salt concentrate was piped under pressure into a stainless steel high pressure autoclave which had been purged previously with nitrogen. In this reactor, which contained a stirrer for agitation, the pressure was immediately raised to 250 pounds per square inch gauge and the temperature was raised to 220° C. The steam was removed until the polymer melt temperature reached 243° C. At this point the reactor pressure was gradually reduced over a 25 minute period to atmospheric pressure and the polymer melt allowed to equilibrate for 30 minutes at 278° C.

This finished polymer so produced was melt spun at 280° C. through a 13 hole spinnerette yielding white 75 multifilament yarns. These yarns were drawn over hot

pins (90° C.) at a maximum draw ratio of 5.65 times their original length.

Dyeing of these yarns was carried out by immersing in an acid dye bath containing 3 percent, based on the weight of the yarn, of Scarlet 4RA Conc. CF (C.I. Acid Red 18) and 1.2 percent formic acid. The weight ratio of dye bath to fiber was maintained at 40:1 and dyeing was conducted for 2 hours at 100° C. and at a pH of 3.1. These yarns absorbed 1.25 percent dyestuff.

#### EXAMPLE II

Di(potassium sulfonate)-naphthalene-2-carboxylic acid was prepared by treating 100 grams of 2-naphthoic acid with 752 grams of 15 percent fuming sulfuric acid for 3 hours at 100° C. The reaction product was then added to 1000 grams of ice followed by slow addition of 250 grams of potassium bicarbonate. A precipitated product formed which was redissolved by adding 3 liters of water and heating the solution to 70° C. followed by treatment with 2 grams of activated charcoal. To the hot filtered solution was then added 225 grams of potassium chloride and precipitation of the finely divided white product, di(potassium sulfonate)-naphthalene-2-carboxylic acid, occurred. The product was filtered off and purified by redissolving in 2300 cc. of water at 70° C. followed by treatment with 1 gram of activated charcoal. After filtration while hot, 100 grams of potassium chloride was added whereupon the product precipitated in the form of finely divided white particles which, after cooling, were isolated by filtration.

The procedure of Example I was repeated with the exception that the above-prepared di(potassium sulfonate)-naphthalene-2-carboxylic acid in an amount sufficient to provide a finished polyhexamethylene adipamide containing 0.555 mole percent additive, was added along with the salt into the autoclave. This modified nylon polymer thus produced was melt spun at 280° C. through a 13-hole spinnerette yielding white multifilament yarns. These yarns were drawn over hot pins (90° C.) at a maximum draw ratio of 4.60 times their original length. These yarns were found to absorb 0.36 percent Scarlet 4RA Conc. CF (C. I. Acid Red 18) acid dye stuff when dyed under identical procedure and dye bath composition as outlined in Example I.

#### EXAMPLE III

The procedure of Example II was repeated with the exception that the additive employed was potassium-3,5-dicarboxybenzene sulfonate which is described in U.S. Patent 3,039,990. The yarn thus produced when treated under identical conditions as employed in Example II was found to absorb 0.80 percent Scarlet 4RA Conc. CF (C. I. Acid Red 18).

#### EXAMPLES IV-VI

The procedures outlined in the above examples were repeated with the exception of the particular additive employed and in the amount in which it was employed. The results obtained are illustrated in Table I.

TABLE I

| Additive                                                              | Mole<br>Percent<br>in<br>Polymer | Amount<br>of Dye<br>Absorption | Increase Dye-Resist.               |                                     |
|-----------------------------------------------------------------------|----------------------------------|--------------------------------|------------------------------------|-------------------------------------|
|                                                                       |                                  |                                | Ex. IV<br>vs.<br>Ex. V,<br>Percent | Ex. IV<br>vs.<br>Ex. VI,<br>Percent |
| Example:                                                              |                                  |                                |                                    |                                     |
| IV (a).....Di(potassium sulfonate)-naphthalene-2-carboxylic acid..... | 0.139                            | 0.71                           | 38.0                               | 34.0                                |
| IV (b).....do.....                                                    | 0.780                            | 0.21                           | 147.9                              | 133.3                               |
| V (a).....Potassium-3,5-dicarboxybenzene sulfonate.....               | 0.139                            | 0.98                           | .....                              | .....                               |
| V (b).....do.....                                                     | 0.780                            | 0.52                           | .....                              | .....                               |
| VI (a).....3-sulfobenzoic acid monosodium salt.....                   | 0.139                            | 0.94                           | .....                              | .....                               |
| VI (b).....do.....                                                    | 0.780                            | 0.49                           | .....                              | .....                               |

These experimental findings clearly show the pronounced superiority of the additives of this invention over the difunctional monosulfonate salt and the monofunctional monosulfonate salt when used in corresponding amounts. Besides the increased acid dye resistance indicated in Table I, it should be noted that the additive em-

ployed in Example II exhibited an increase acid dye resistance of nearly 122 percent over the additive employed in Example III.

#### EXAMPLE VII

5 Acid dye-resist poly-epsilon-caproamide was prepared by introducing 100 grams of epsilon-caprolactam and 1.94 grams of di(potassium sulfonate)-naphthalene-2-carboxylic acid into a stainless steel high pressure autoclave. After purging with nitrogen the autoclave was pressurized 10 to 250 pounds per square inch gauge and the temperature was raised to 250° C. while steam was continually removed. At this point the pressure was gradually reduced over a 25 minute period to atmospheric pressure and the temperature of the molten polymer reached 265° C. The 15 vacuum cycle was then applied to the autoclave by gradually lowering the pressure over a 30 minute period to 25 inches of mercury, and the polymer melt allowed to equilibrate under these conditions for 10 minutes before returning the autoclave to atmospheric pressure by allowing nitrogen to bleed back into the system. The polymer was immediately melt spun at 265° C. directly from the 20 autoclave as 13 multifilament white yarn.

The dyeing procedure and conditions outlined in Example I were repeated and these yarns were found to absorb 25 0.60 percent Scarlet 4RA Conc. CF (C. I. Acid Red 18) compared to 1.08 percent absorption which was observed on conventional poly-epsilon-caprylamine yarns containing 0.536 mole percent potassium-3,5-dicarboxybenzene sulfonate which were prepared and dyed under identical 30 conditions.

#### EXAMPLE VIII

Poly-hexamethylene sebacamide modified in accordance with the present invention was prepared by charging a 35 stainless steel evaporator with 0.393 mole of hexamethylene diammonium sebacate dissolved in 20.8 moles of water containing 0.968 gram of di(potassium sulfonate)-naphthalene-2-carboxylic acid. After purging the evaporator with nitrogen the unit was pressurized to 13 pounds 40 per square inch gauge and heated to 137° C. with removal of steam condensate. At this temperature the concentrated salt was then piped under pressure to a high pressure autoclave, which was previously purged with nitrogen, and the unit pressurized to 250 pounds per square inch gauge 45 and the temperature raised to 230° C. with the continual removal of steam. At this temperature the pressure in the autoclave was gradually reduced over a 25 minute period to atmospheric pressure while the polymer melt temperature was raised to 265° C. The melt was then allowed to 50 stand and equilibrate for a period of 30 minutes prior to melt spinning at 265° C. directly from the autoclave through a 13 hole spinnerette yielding white multifilament yarn.

The spun yarns were drawn over hot pins (90° C.) at a maximum draw ratio of 4.50 times their original length. The yarns were dyed in accordance with the procedure and conditions outlined in Example I, and were found to

70 absorb 0.39 Scarlet 4RA Conc. CF (C. I. Acid Red 18). Yarns prepared in an identical manner with the exception that potassium-3,5-dicarboxybenzene sulfonate was the additive used were found to absorb 0.70 percent of the same dye. It will be observed that yarns containing the additive of the present invention exhibit an increase in acid

dye-resist properties of 79.5 percent over yarns containing additives disclosed by the prior art.

## EXAMPLE IX

Di(sulfonic acid)-naphthalene-2-carboxylic acid was prepared by treating a dilute aqueous solution of di(potassium sulfonate)-naphthalene-2-carboxylic acid with a cation exchange resin in an ion-exchange column. The treated solution was then evaporated to dryness yielding a white product, di(sulfonic acid)-naphthalene-2-carboxylic acid. The preparation of modified poly-hexamethylene adipamide containing 0.60 mole percent of di(sulfonic acid)-naphthalene-2-carboxylic acid was carried out by the same procedure and conditions described in Example I. The additive was incorporated into the polymer preparation in the same method as described in Example II.

The resultant polymer was melt spun at 280° C. directly from the preparatory autoclave into 13 multifilament white yarns which were drawn at a maximum draw ratio of 5.70 times their original length.

These yarns were found to absorb 0.73 percent of Scarlet 4RA Conc. CF (C.I. Acid Red 18) when dyed according to procedure and conditions outlined in Example I. This dye absorption represents very nearly 41.6 percent improvement in the dye-resist character over conventional polyhexamethylene adipamide which absorbs 1.25 percent of the same dye.

## EXAMPLE X

Di(ammonium sulfonate)-naphthalene - 2 - carboxylic acid was prepared by reacting 1 mole ratio of di(sulfonic acid)-naphthalene-2-carboxylic acid with 2 mole ratios of ammonium hydroxide in an aqueous solution and the diammonium salt product allowed to remain in solution. Modified polyhexamethylene adipamide containing 0.60 mole percent of the diammonium salt was carried out by the same procedure and conditions described in Example I. The additive was incorporated into the polymer preparation in the same manner as described in Example II.

The resultant polymer was melt spun at 280° C. into 13 multifilament white yarns which could be cold drawn. These yarns were found to absorb 0.67 percent Scarlet 4RA Conc. CF (C.I. Acid Red 18) when dyed according to procedures and conditions outlined in Example I. This dye absorption represents very nearly 46.4 percent improvement in the acid dye resist character over the standard polyhexamethylene adipamide yarns which absorb 1.25 percent of the same dye.

As can be seen from the above results, fibers made from the polycarbonamides of the present invention all possess a resistance to acid type dyes. This enables manufacturers to produce fibers having the same basic polycarbonamide molecular structure as conventional polycarbonamides but different affinities for acid dyes. This in turn offers dyeing diversification for fabric color-on-white effects and tone-on-tone effects heretofore not readily obtainable.

We claim:

1. A fiber-forming synthetic linear polycarbonamide wherein recurring carbonamide linkages are an integral part of the polymer chain and containing as a component part of the polymer chain between about 0.1 and 2.0 mole percentage, based on the molecular weight of the polycarbonamide of units of the structure:



wherein Z is a member of the class consisting of



X is a member of the class consisting of hydrogen and lower alkyl, M is a member of the class consisting of hydrogen, the ammonium radical and an alkali metal and n is a number from zero to 6 inclusive with the proviso that when Z is



then n is at least 1.

2. The fiber-forming synthetic linear polycarbonamide as set forth in claim 1 wherein the polycarbonamide is poly-hexamethylene adipamide.

3. The fiber-forming synthetic linear polycarbonamide as set forth in claim 1 wherein the polycarbonamide is poly-epsilon-caproamide.

4. The fiber-forming synthetic linear polycarbonamide as set forth in claim 1 wherein the polycarbonamide is poly-hexamethylene sebacamide.

5. A fiber-forming synthetic linear polycarbonamide wherein recurring carbonamide linkages are an integral part of the polymer chain and containing as a component part of the polymer chain between about 0.05 and 2.0 mole percentage based on the molecular weight of the polycarbonamide of units of the structure:



6. Polyhexamethylene adipamide containing as a component part of the polymer chain between about 0.05 and 2.0 mole percentage based on the molecular weight of the polyhexamethylene adipamide of units of the structure:



7. Polyhexamethylene adipamide containing as a component part of the polymer chain between about 0.05 and 2.0 mole percentage, based on the molecular weight of the polyhexamethylene adipamide of units of the structure:



8. Polyhexamethylene adipamide containing as a component part of the polymer chain between about 0.05 and

9

2.0 mole percentage, based on the molecular weight of the polyhexamethylene adipamide of units of the structure:



9. Poly-epsilon-caproamide containing as a component part of the polymer chain between about 0.05 and 2.0 mole percentage, based on the molecular weight of the poly-epsilon-caproamide of units of the structure:



10. Polyhexamethylene sebacamide containing as a component part of the polymer chain between about 0.05 and 2.0 mole percentage based on the molecular weight

5

of the polyhexamethylene sebacamide of units of the structure:



10

10. 11. A textile fiber consisting essentially of the poly-carbonamide as defined in claim 1.

## References Cited

## UNITED STATES PATENTS

- |    |           |        |              |       |        |
|----|-----------|--------|--------------|-------|--------|
| 15 | 3,039,990 | 6/1962 | Huffman      | ----- | 260—78 |
|    | 3,142,662 | 7/1964 | Huffman      | ----- | 260—78 |
|    | 3,184,436 | 5/1965 | Magat        | ----- | 260—78 |
|    | 3,296,204 | 1/1967 | Caldwell     | ----- | 260—78 |
| 20 | 3,328,484 | 6/1967 | Lugaz et al. | ----- | 260—78 |

WILLIAM H. SHORT, Primary Examiner.

H. D. ANDERSON, Assistant Examiner.

25

U.S. Cl. X.R.

260—78; 8—55; 57—140